

Patented Aug. 25, 1953

2,650,172

# UNITED STATES PATENT OFFICE

2,650,172

## MOISTUREPROOFING OF NONFIBROUS CELLULOSIC MATERIAL

William O. Brillhart, Fredericksburg, Va., assignor to American Viscose Corporation, Wilmington, Del., a corporation of Delaware

No Drawing. Application January 21, 1949,  
Serial No. 72,065

12 Claims. (Cl. 117—76)

**1** This invention relates to improvements in non-fibrous cellulosic articles. More particularly it relates to the treatment of regenerated cellulose sheets or films with an aqueous alkaline medium containing an anchoring agent for film-forming surface coatings whereby slightly alkaline sheets or films which are not embrittled by age, and to which the surface coating firmly adheres, are obtained.

It is desirable, in the manufacture of sheets and films of hydrophilic cellulosic materials, such as regenerated cellulose and cellulose ethers and esters containing free hydroxyl groups, to provide the sheets and films with a surface coating for improving certain characteristics of the cellulosic article, such as its moistureproof, vapor proof, and/or heat sealing characteristics. A number of substances and compositions have been proposed for this purpose. However, it has been recognized that when the treated sheets are used to package materials of high moisture content, or come in contact with an atmosphere of high humidity or a medium actually containing liquid water, the cellulosic base tends to swell, and the surface coating tends to loosen and slough off. A number of different materials have been proposed for use as an intermediate anchoring agent between the hydrophilic cellulose and the surface coating. Some of these anchoring agents have had the disadvantage that they are acidic or revert to an acidic condition when the cellulosic article is dried after it has been treated with them. This is undesirable because cellulosic articles which comprise an acid tend to become brittle and fragile on ageing due to acid degradation of the cellulose. Such articles cannot be stored safely for any appreciable period of time. In order to avoid this difficulty it is necessary to treat the article, after application of the anchoring agent, to bring it to neutral or alkaline condition.

Other anchoring agents have had the disadvantage that they must be applied from organic solvents, entailing expensive solvent recovery processes.

The principal object of this invention is to produce cellulosic articles, for example sheets or films, which are slightly alkaline as produced, and which can be given a top or surface coating of a film-forming substance or composition which imparts moistureproof, vapor proof, and/or heat-sealing characteristics to the cellulosic article, whereby the surface coating is firmly anchored to the cellulosic article and is resistant to loosening or sloughing off when the article is exposed to moisture. Another object is to provide an improved method for conditioning cellulosic articles for reception of a surface or top coating wherein the anchoring agent is applied from aqueous alkaline medium. Another object

**2** is to produce cellulosic articles which adhere firmly to film-forming moistureproofing agents or compositions in contact with moisture and which do not become brittle with use or on long storing either before or after application of the moistureproofing agent. Other objects of the invention are to provide a simple, practical method of applying an anchoring agent to cellulosic articles from an alkaline solution which does not require any change in conventional processes for manufacturing such articles. Other objects will appear hereinafter.

The objects of the invention are accomplished by treating cellulosic articles such as sheets, films, pellicles, tubes, filaments, etc., with aqueous alkaline medium containing a resin comprising a polymerization product of styrene and maleic anhydride containing 50 mol per cent of styrene in the polymer molecule, in the form of a water-soluble salt of an alkaline agent selected from the group consisting of ammonia and amines having up to four carbons, and thereafter heating the treated cellulosic article to dry the article and insolubilize the resin under controlled conditions such that the amount of alkaline agent such as the amine or ammonia volatilized during the heating and insolubilizing step is not sufficient to effect conversion of the resin to the free acid state. In this way, cellulosic articles which are slightly alkaline are obtained.

The cellulosic articles may be of regenerated cellulose prepared from solutions of cellulose xanthate or cuprammonium cellulose, or they may be of a cellulose ester or ether, such as cellulose acetate, cellulose nitrate, ethyl cellulose, methyl cellulose, etc. which materials contain free hydroxyl groups and are hydrophilic in character.

In the preferred embodiment of the invention, an ammonium or amine salt of the styrene-maleic anhydride polymerization product is incorporated directly in the aqueous softening bath, such as the glycerol bath, on the casting machine for producing regenerated cellulose sheets, and thus the anchoring agent is applied to the gel sheet as it passes through the glycerol bath, after the sheet has been purified and washed, while it is in substantially neutral, water-laden condition, and prior to initial drying thereof. The sheet is then dried under controlled conditions of time and temperature such that the styrene-maleic anhydride polymerization product is insolubilized without sufficient evolution of ammonia or amine to convert the anchoring agent to the acid condition. This curing of the resin without reversion thereof to the free acid state is accomplished by drying the impregnated sheet or film and simultaneously curing the resin at relatively low temperatures of 50-80° C. for a short period of from 1 to 5

## 3

minutes. After the sheet or film has been dried, the heating may be continued for from 0.5 to 1.0 minute, if desired, without volatilizing sufficient ammonia or amine to convert the resin to an acid condition. The finished dried cellulosic sheet 5 which is slightly alkaline is then ready for storing or use and will be found to retain its strength and flexibility for long periods of time. It may be given a surface coating of a film-forming substance or composition for rendering 10 it moistureproof, or otherwise modifying or improving its characteristics, immediately after it is produced or at any time subsequent to its production and such coating will be found to adhere tenaciously to the sheet for a substantial 15 period of time even when it is in direct contact with water.

The anchoring agent is produced by the polymerization of maleic anhydride and styrene in equimolar proportions, and may be obtained by 20 dissolving or suspending maleic anhydride in styrene and heating the mixture until the monomers are interpolymerized and a polymeric product containing 50 mol per cent of styrene in the polymer molecule is produced, recovering 25 the polymerization product, purifying it by precipitation with acid from an alkaline solution, and then reacting it with ammonia or an organic amine containing up to four carbons, to produce the ammonium or amine salt.

In order to specifically illustrate the invention, the following examples in which parts are by weight unless otherwise indicated are given.

## Example I

A sheet of gel regenerated cellulose which had been desulfured, bleached, and washed free of impurities on the casting machine was passed, prior to drying thereof, through an aqueous bath containing 5% of glycerol as plasticizer, and 0.1% of an ammonium salt of a heteropolymer of styrene and maleic anhydride containing 50 mol per cent of styrene in the polymer molecule, at room temperature. The excess treating solution was removed from the sheet by squeeze rolls and the sheet was heated at 80° C. for 5 minutes, to dry the sheet and 35 insolubilize the resin.

Under the stated conditions, some ammonia was evolved with, it is believed, the formation of cross-linked amides and imides, but the amount of ammonia so volatilized was insufficient to cause the anchoring material to revert to acidic character. The resin was applied 50 and cured under alkaline conditions, and the finished sheet was slightly alkaline.

The resin-treated sheet is coated with a moistureproof lacquer of the following illustrative composition:

|                            | Percent |
|----------------------------|---------|
| Nitrocellulose             | 6.75    |
| Gum dammar                 | 1.64    |
| Dibutyl phthalate          | 2.80    |
| Paraffin (M. P. 60-61° C.) | 0.48    |
| Zinc stearate              | 0.15    |
| Ethyl acetate              | 56.34   |
| Toluene                    | 28.53   |
| Ethanol                    | 3.20    |
| Acetone                    | 0.11    |

The sheet is passed through the moisture-proofing lacquer, the excess lacquer is removed by scraping or by any suitable means, and the sheet dried at temperatures above the melting point of the wax present in the lacquer. The sheet is then cooled, and humidified, after which 75

## 4

it will be found to adhere firmly to the moisture-proof surface coating for appreciable periods of time even in direct contact with moisture or water.

## Example II

A sheet of gel regenerated cellulose which had been desulfured, bleached and washed free of impurities on the casting machine was passed, prior to any drying thereof, through an aqueous alkaline medium containing 5% of glycerol as plasticizer, 0.2% of an ammonium salt of a heteropolymer of styrene and maleic anhydride containing 50 mol per cent of styrene in the polymer molecule, and 0.01% of trimethylbenzyl ammonium chloride, at room temperature. The excess treating medium was removed from the sheet by squeeze rolls and the sheet was then heated to 70° C. for 3 minutes to dry the sheet and insolubilize the resin.

## Example III

A sheet of gel regenerated cellulose which had been desulfured, bleached and washed free of impurities on the casting machine was passed, prior to any drying thereof, through an aqueous alkaline medium containing 6% of glycerol as plasticizer and 0.4% of the ethyl amine salt of a heteropolymer of styrene and maleic anhydride containing 50 mol per cent of styrene in the polymer molecule, at room temperature. The excess treating medium was removed from the sheet by squeeze rolls and the sheet was heated at 75° C. for 4 minutes to dry the sheet and insolubilize the resin. The dried sheet was 30 slightly alkaline.

The quantity of ammonium or amine salt of the styrene-maleic anhydride polymerization product used may vary, but generally such salts are used in an amount of from 0.1 to 5% by weight 40 of the treating solution.

As is evident from Example II above, the aqueous medium containing the anchoring agent applied at the plasticizing stage may also contain small amounts, preferably from 0.1 to 2%, of a quaternary ammonium salt which apparently catalyzes the insolubilization of the heteropolymer. The exact manner in which the quaternary ammonium salt functions is not clear. However, when the anchoring resin contains such agents it is fixed more firmly to the cellulosic base, and in shorter periods of heating, than when the quaternary ammonium salt is omitted. Examples of other quaternary ammonium salts which may be used are triethyl 50 benzyl ammonium chloride, octyloxymethyl diethyl allyl ammonium chloride, isobutyloxy-methyl dimethyl-B-methylallyl ammonium chloride, etc.

As a result of the heating step, the anchoring agent is insolubilized. The cellulosic sheets or films obtained in accordance with this invention may be coated with any suitable film-forming agent or composition such as, for example, a moistureproofing composition comprising a flowable solution of a cellulose derivative, a wax, or wax-like material, a resin or blending agent, and a plasticizer, or with any other film-forming material or composition for improving or modifying the properties of the cellulose base. 60 Surface or top coatings which normally do not adhere strongly to cellulosic sheets or the like, especially in contact with moisture, are firmly anchored to the cellulosic article through the resinous anchoring agent and adhere to the cellulose base even when the article is exposed 65 to moisture.

rectly to moisture. The treated article, which is alkaline in character, retains its flexibility and toughness and does not become brittle with age.

Since variations and modifications may be made in the invention as specifically exemplified herein, any such variations or modifications which conform to the spirit of the invention are intended to be included within the scope of the claims.

I claim:

1. In the production of cellulosic articles the improvement which comprises applying to the article while it is in the form of a wet gel prior to initial drying thereof as a step in its manufacture, an aqueous alkaline medium containing a water-soluble salt of a polymerization product of styrene and maleic anhydride containing about 50 mol per cent of styrene in the polymer molecule, said salt being formed with an alkaline agent selected from the group consisting of ammonia and amines having up to four carbons, removing excess treating medium, and thereafter heating the cellulosic article under controlled conditions of temperature and time to dry the article and insolubilize the polymerization product without volatilizing sufficient alkaline agent to convert the polymerization product to an acid condition, and then applying to the article a film-forming moistureproofing agent.

2. A method as in claim 1 wherein the aqueous alkaline medium also contains a quaternary ammonium salt as a catalyst for said insolubilization.

3. A method as in claim 1 wherein the aqueous alkaline medium also contains a plasticizer for the cellulosic article and a quaternary ammonium salt as a catalyst for said insolubilization.

4. A method for the production of a moisture-proof cellulosic article which comprises applying to a hydrophilic cellulosic article, while it is in the form of a wet gel prior to initial drying thereof as a step in its manufacture, an aqueous alkaline medium comprising an anchoring agent for film-forming moistureproofing materials, said anchoring agent being a water-soluble salt of a polymerization product of styrene and maleic anhydride containing about 50 mol per cent of styrene in the polymer molecule, said salt being formed with an alkaline agent selected from the group consisting of ammonia and amines having up to four carbons, removing excess treating medium, heating the treated article to a temperature of from 50 to 80° C. for from 1 to 6 minutes to dry the article and insolubilize the polymerization product without volatilizing sufficient alkaline agent to convert the polymerization product to an acid condition, and then applying to the article a film-forming moistureproofing agent.

5. A method as in claim 4 wherein the cellulosic article comprises regenerated cellulose.

6. A method as in claim 4 wherein the cellulosic article comprises regenerated cellulose and

the aqueous alkaline medium also contains a plasticizing agent for the cellulose.

7. A method as in claim 4 wherein the cellulosic article comprises regenerated cellulose and the aqueous alkaline medium also contains glycerol as a plasticizing agent for the cellulose.

8. A method as in claim 4 wherein the cellulosic article comprises regenerated cellulose and the aqueous alkaline medium also contains a quaternary ammonium salt as a catalyst for said insolubilization.

9. A method as in claim 4 wherein the cellulosic article comprises regenerated cellulose and the aqueous alkaline medium also contains a plasticizer for the cellulosic article and a quaternary ammonium salt as a catalyst for said insolubilization.

10. A composite film comprising a cellulosic base, a moistureproof coating, and, disposed between the base and the moistureproof coating, an intermediate coating of an insoluble resin, said resin being the insolubilized product of a water-soluble salt of a styrene-maleic anhydride polymerization product containing about 50 mol per cent of styrene in the polymer molecule, said salt being formed with an alkaline agent selected from the group consisting of ammonia and amines having up to four carbons, said resin being in the insolubilized condition resulting from the heating of the water-soluble salt without volatilizing sufficient alkaline agent to convert the polymerization product to an acid condition.

11. A composite film as defined in claim 10 wherein the cellulosic base is a sheet of regenerated cellulose.

12. A composite film as defined in claim 11 wherein the sheet of regenerated cellulose is plasticized with glycerol.

WILLIAM O. BRILLHART.

References Cited in the file of this patent  
UNITED STATES PATENTS

| Number    | Name               | Date          |
|-----------|--------------------|---------------|
| 1,976,679 | Fikentscher et al. | Oct. 9, 1934  |
| 2,047,398 | Voss et al.        | July 14, 1938 |
| 2,168,535 | Nuesslein et al.   | Aug. 8, 1939  |
| 2,252,091 | Muller et al.      | Aug. 12, 1941 |
| 2,327,760 | Bestian et al.     | Aug. 24, 1943 |
| 2,341,413 | Pense et al.       | Feb. 8, 1944  |
| 2,356,879 | Pense et al.       | Aug. 29, 1944 |
| 2,394,009 | Pollard            | Feb. 5, 1946  |
| 2,432,542 | Ritzl              | Dec. 16, 1947 |
| 2,467,436 | Lanning            | Apr. 19, 1949 |
| 2,469,407 | Powers et al.      | May 10, 1949  |
| 2,469,408 | Powers et al.      | May 10, 1949  |
| 2,469,409 | Powers et al.      | May 10, 1949  |
| 2,486,804 | Seynor et al.      | Nov. 1, 1949  |

FOREIGN PATENTS

| Number  | Country       | Date          |
|---------|---------------|---------------|
| 466,817 | Great Britain | June 7, 1937  |
| 497,335 | Great Britain | Dec. 15, 1938 |